

J. F. WHITE,

BAG FOR CONTAINING CEMENT AND METHOD OF MAKING SAME.

APPLICATION FILED APR. 17, 1916.

1,195,311.

Patented Aug. 22, 1916.



Witness:

Jas. E. Hutchinson:

By

Inventor:

John F. White,  
Grand Island, Attorneys:

# UNITED STATES PATENT OFFICE.

JOHN F. WHITE, OF CHICAGO, ILLINOIS.

## BAG FOR CONTAINING CEMENT AND METHOD OF MAKING SAME.

1,195,311.

Specification of Letters Patent. Patented Aug. 22, 1916.

Application filed April 17, 1916. Serial No. 91,678.

To all whom it may concern:

Be it known that I, JOHN F. WHITE, a citizen of the United States, residing at Chicago, in the county of Cook and State of Illinois, have invented certain new and useful Improvements in Bags for Containing Cement and Methods of Making Same, of which the following is a specification, reference being had therein to the accompanying drawing.

This invention relates to an improved method of producing cement bags and in the article produced thereby.

Heretofore many attempts have been made to produce economically, a cement bag, which could be reemployed after use and which could be economically manufactured. Owing to the now recognized importance of the industry, it has been the desire of manufacturers to secure a bag which would receive ground cement and retain the same without sifting through the meshes of the cloth or canvas and which would prevent moisture from entering through the sides of the bag. The present invention is designed to meet this demand and is produced by the following process. A strip of canvas of a width substantially the required length of a bag is coated in any convenient manner with a coating of a hydrocarbon compound having an asphalt base. In this particular I have found that petroleum residuum approximately seventy per cent., mixed with thirty parts asphaltum or the equivalent of these two substances and subjected to heat, can be applied directly to the surface of the bag material. In this condition the surface coating is tacky and sticky. After the material has been properly coated with a layer of the substance, it is carried over an edge-forming roll where the edges of the material are turned to form a hem, the turning of the material being in the direction of the coated surface. By passing over the roll under tension the turned-over edge is drawn tightly onto the sticky surface of the body of the fabric and is there held or set, so as to become well secured in its turned-over or hemmed position. This turning-over of the edge of the fabric is conveniently along the selvage and represents a reinforced edge to the bag presently to be described.

The material is carried from the roll a short distance and thereafter has applied to its coated surface powdered talc or other

substance which will render the surface treated nonadherent. In this condition the material is allowed to dry for a period of time and then is ready for use in the manufacture of the bag.

In the drawings: Figure 1 is a diagrammatic view of an apparatus employed in carrying out the method, and Fig. 2 is a detail view of the bag.

In the accompanying drawing there is shown diagrammatically the hemming roll at A.

B represents the tensioned fabric passing over the roll, its untreated face being against the roll.

C represents a turnover pin which may be held by the hand of the operator which causes the selvage of the material to be turned onto the tacky treated surface of the same, and in this condition, owing to the increased thickness of the material at the hem, the turned-over portion is drawn tightly onto the roll and there set and held, thereby avoiding the necessity of a presser roll or other pressing means.

C' designates the powdering box through which the material passes.

In producing the article it has been found heretofore that when the edges of the open mouth of the bag have been stitched, the lock-stitch usually being employed, a very thick portion is present for the pressure foot of the machine to pass over, and again it has been found necessary to employ the step of stitching prior to the closing in of the sides and bottom of the bag. In the present method it is only necessary to take the material and place the side and bottom edges together and lockstitch the edges in the usual manner. The bag is then turned with the treated side in, leaving the hem in a condition where it will maintain its position while the inside of the bag has the desired ~~containing~~ <sup>protecting</sup> the same substantially impervious. Inasmuch as the coating material is more or less tacky and soft, as distinguished from a hard or nontacky material, the cement as it comes in contact with the surface adds additional powder thereto and thereby renders the bag useful for subsequent use as the treated surfaces will not then adhere to each other.

I desire it understood that the invention is not limited to the use of the particular material herein specified.

60

65

70

75

80

85

90

95

100

105

110

Having thus described the invention, what is claimed as new and desired to be secured by Letters Patent is:

1. The art of producing water-repellent bag material consisting in applying to the surface of woven fabric a water-proofing tacky substance of a hydrocarbon nature turning the edge of the fabric over onto the adjacent tacky surface of the body of the same, causing the turned-over edge to be tightly drawn onto the surface, and subsequently coating the surface with powdered substance.
2. The art of producing a bag making fabric consisting in applying to one surface of the fabric a hydrocarbon substance having an asphaltum base, and turning the edge of the fabric over onto the adjacent treated surface of the body thereof and tightly forcing the turned-over edge onto the body, and applying to the treated surface a powdered substance.
3. The art of hemming the edge of fabric having a water repellent adhesive surface coating, consisting in folding the edge of the fabric over onto the adjacent treated

surface thereof and by pressure exerted lengthwise of the fabric to set the said over-turned edge tightly onto the treated face of the fabric.

30

4. A cement bag having its inner surface coated with a water-repellent substance, and the edge of the open part thereof being turned down onto the adjacent part of the body to form a hem and held in its turned-down position by the treating substance, substantially as described.

5. A cement bag having its inner surface coated with a water-repellent substance, and the edge of the open part thereof being turned down onto the adjacent part of the body to form a hem and held in its turned-down position by the treating substance, the inner surface of the bag being coated with a powdered substance, substantially as described.

In testimony whereof I hereunto affix my signature in the presence of two witnesses.

JOHN F. WHITE.

Witnesses:

WALTER W. HISS,  
HELEN A. NYMAN.